

Aug. 28, 1962

H. P. FRY, JR

3,051,606

RAYON FABRIC REINFORCED LAMINATED SHEET

Filed Nov. 26, 1958



Fig-1



Fig-2

# United States Patent Office

3,051,606

Patented Aug. 28, 1962

1

3,051,606

## RAYON FABRIC REINFORCED LAMINATED SHEET

Horace P. Fry, Jr., West Chester, Pa., assignor to American Viscose Corporation, Philadelphia, Pa., a corporation of Delaware

Filed Nov. 26, 1958, Ser. No. 776,587

2 Claims. (Cl. 156—229)

This invention relates to rayon fabric reinforced laminated sheets and more particularly to an improved method of reinforcing paper or the like with a lamina of high tenacity rayon fabric. More specifically, the present invention deals with the manner in which the rayon fabric, which is preferably in the form of an open-mesh, non-woven scrim, is acted upon at the time of laminating it to a sheet material so as to reduce the inherent extensibility of the fabric to a value approximating that of the sheet material.

The usual continuous filament viscose rayon yarn, unless highly twisted, has an extensibility of approximately 18% when dry and 22% when wet before its full strength is realized and the yarn breaks. This high extensibility can be considerably reduced, say to about 8% or even less, if during initial manufacture or subsequently, the yarn is subjected to a slashing operation wherein the yarn is wetted and then held under tension while drying. However, the reduced extensibility brought about by slashing is destroyed if the yarn is subsequently gotten wet and allowed to dry in a relaxed or untensioned condition and consequently slashing is ordinarily only employed when the yarn is to be used in a manner wherein it is protected from water, as for example, for tire cord.

Open-mesh fabric known as scrim, which may be either woven or nonwoven, has a wide variety of uses. Obviously, in the case of non-woven scrim, the yarns making up the fabric must be secured together at their crossing points in order to hold the fabric together and this is customarily accomplished by means of an adhesive. It is also customary to employ an adhesive to secure the yarns together at their crossing points in woven scrim, especially in the case of wide mesh scrim. Because the individual threads or yarns of scrim are not closely packed together as they are in a closely woven fabric, the scrim has an extensibility substantially equal to that of individual yarns of which it is formed. Thus, scrim formed of ordinary, unslashed, low-twist viscose rayon yarn has an extensibility of approximately 18% when dry and 22% when wet. Scrim formed of slashed rayon yarns has a much lower extensibility but the adhesive employed must not contain water or be applied as a water emulsion or suspension unless the individual yarns are maintained under tension until the fabric is completely dry for otherwise the low-extensibility characteristic of the yarn is destroyed, as mentioned above. While there are certain volatile adhesives which may be used which do not impair the low-extensibility of the yarn, these create undesirable and expensive problems in connection with solvent recovery, ventilation, fire hazard, etc. On the other hand, when an aqueous adhesive liquid is employed, the mechanisms necessary to maintain the yarn under tension until dry are complicated and the fabric-forming operation generally has to proceed at a slower rate. While a scrim of low extensibility is ideally suited as a reinforcing lamina for paper or other sheet material, the above-mentioned problems in connection with forming the scrim of a low extensibility rayon yarn have limited its use for this purpose. This use has been further restricted by the necessity for employing volatile, non-aqueous adhesives when laminating the scrim to the paper.

2

It is an object of the present invention to provide an improved method of laminating an open-mesh rayon fabric to a sheet of paper or like material in such manner that the fabric will have an extensibility substantially equal to that of the material to which it is laminated whereby the composite sheet will have a breaking strength substantially equal to the combined breaking strengths of the fabric and the material to which it is laminated.

It is a further object of this invention to provide a method of laminating an open-mesh rayon fabric to a sheet of another material in such manner that the fabric and the sheet to which it is laminated will have substantially the same extensibility and wherein the fabric is formed of ordinary unstrained rayon yarn.

It is a still further object of this invention to permit a highly extensible rayon yarn to be used for forming a fabric which is subsequently used as a reinforcing lamina for sheet material.

Another object of the invention is to provide a laminating technique which permits the use of an aqueous adhesive liquid for reinforcingly adhering an open-mesh rayon fabric to a sheet of paper.

Still another object is to provide a method of reinforcing various flexible sheet materials with an open-mesh rayon fabric which permits ordinary unstrained yarn to be used to form the fabric to thus effect substantial economy in manufacture.

Other and further objects, features and advantages of the invention will become apparent as the description thereof proceeds.

Referring now to the drawing:

FIGURE 1 is a plan view of a form of apparatus suitable for use in practicing the invention; and

FIGURE 2 is a side elevational view of the apparatus.

In the drawing, the scrim, an open-mesh woven or non-woven fabric, is indicated at 10 and two lengths of sheet material such as paper or the like, between which the scrim is to be laminated, are indicated at 11 and 12. Methods and apparatus for manufacturing scrim are well known in the art and need not be described herein but it is to be noted that in accordance with this invention, it may be formed of ordinary, unstrained, continuous filament, low twist viscose rayon yarn and in fact in order to obtain the full advantage of this invention it is preferably formed of such yarn. However, certain advantages of the present invention may be realized when the scrim is formed of so-called high-tenacity yarn, that is to say, yarn which has been dried without allowing it to shrink so as to reduce the extensibility thereof and it is therefore within the purview of the invention to form the scrim of this type of yarn.

As previously noted, the ordinary, unstrained rayon yarn has an extensibility of approximately 18% when dry and the scrim formed of such yarn has a like degree of extensibility. In order for the scrim to effectively reinforce the paper or other material with which it is laminated, it is necessary that the extensibility of the scrim and the paper be substantially the same so that when a strain is applied to the laminated structure the full combined strength of both materials may be realized before either breaks. Now the paper or other material 11 and 12 will normally have very considerably less extensibility than the scrim and according to the present invention the extensibilities of the two materials are equalized by stretching the scrim, wetting it and drying it under tension to reduce the extensibility of the scrim to that of the paper. For example, assuming that the paper is capable of stretching 4% before bursting; the scrim, if it inherently has 18% extensibility will be stretched 14%, wetted and dried without allowing it to shrink and thereafter so long as it remains dry it will have an extensibility of only 4%. It will be under-

stood that these percentages are used only by way of example and that according to the teaching of this invention it is necessary to determine the actual inherent extensibility of the particular scrim and the particular sheet material with which it is to be laminated and then stretch the scrim accordingly. This stretching, wetting and drying under strain is not performed as a separate operation as is the case when slashing yarn but is performed simultaneously and as an integral part of the laminating process.

The scrim 10 is led from a roll, not shown, and pulled forward by a pair of feed rollers 13 and 14. The feed rollers are driven at a speed sufficiently faster than the speed of the roll from which the scrim is being withdrawn so that the desired amount of stretch is imparted to the scrim in its longitudinal direction. A pair of nip plates 15 and 16 are secured to angularly arranged shafts 17 and 18 respectively, located at one side of the scrim and a similar arrangement of nip plates generally indicated at 19 is mounted at the opposite side of the scrim. The opposite edges of the scrim are directed between the respective pairs of nip plates so that as the scrim is pulled forward by the feed rollers 13 and 14 the opposite edges thereof are grasped by the nip plates which are rotated in a direction and at a speed to transversely stretch the scrim to the predetermined extent equal to the longitudinal stretch.

The two sheets of paper 11 and 12 are directed between the feed rollers 13 and 14 so as to be pulled forward thereby but they are fed from their source at the same speed that they are pulled forward so that there is no stretching of the paper. Spray nozzles 20 and 21 are provided for spraying an aqueous adhesive liquid onto the facing sides of the two paper sheets. The present invention permits the use of a wide range of adhesives as, for example, polyvinyl alcohol, animal glue, carboxymethyl cellulose or an aqueous latex emulsion. At a point very close in time after the spraying on of the adhesive, the adhesive coated faces of the sheets 11 and 12 engage the stretched scrim at the feed rolls 13 and 14. The feed rolls extend for at least the width of the paper sheets so as to hold the scrim in its stretched condition after it is passed beyond the nip plates.

The water in the adhesive liquid moistens the scrim sufficiently that it will retain its increased size and reduced extensibility if held taut until dry. A series of heated pressure drying rolls 22 are located beyond the feed rollers 13 and 14 and the sheets of paper and the scrim are held tightly pressed together as they pass around and between the rolls 22 as shown in FIGURE 2. After leaving the rolls 22 the now laminated sheet 23 may be wound into a roll. The laminated sheet 23 thus comprises two sheets of paper or the like inherently having a reasonably low extensibility between which is adhered the scrim which now has an extensibility substantially equal to that of the paper.

A creped laminated sheet can be made by the process of this invention and this is most advantageously accomplished by using a scrim made from slashed yarn having an extensibility no more than about twice that of the sheets to or between which it is to be laminated. In this case the scrim is stretched both longitudinally and transversely to an extent where its remaining extensibility is substantially equal to that of the paper or the like, but instead of using an aqueous adhesive liquid a non-aqueous adhesive such as asphalt may be employed. As the scrim and the paper pass around and between the rollers 22, the asphalt causes the scrim to adhere to the paper but since no water is applied to the scrim it will have a strong tendency to return to its original dimensions after passing through the rolls 22 and unless the paper or other material between which the scrim is laminated is especially strong, the scrim will return to its

original size and in doing so will crinkle or crepe the paper in all directions. Because of the creping, the extensibility of the paper is greatly increased so that the extensibility of the paper and the scrim are substantially the same.

A creped laminated sheet may also be made by using a scrim formed from a yarn having substantially the same extensibility as that of the sheets with which it is laminated. In this case the scrim is not stretched but is merely fed through the feed rollers 13 and 14 between the other sheets. Of course, the scrim itself will originally be of the same width as the other two sheets. An aqueous adhesive solution is used so that the scrim will have a strong tendency to shrink. However, the scrim is held taut by the feed rollers 13 and 14 and the pressure dryer rolls 22 so that it cannot shrink to an appreciable extent and its extensibility is therefore substantially unchanged. However, unless the paper is especially stiff the scrim will shrink to a small degree and in doing so will crepe the paper in all directions.

Of course, in any of the examples hereinbefore referred to, the scrim need not be located between two sheets but may be adhered to one or both sides of a single sheet of paper or the like.

Having thus described several methods embodying the inventive concept, what is claimed is:

1. The method of making a rayon fabric reinforced laminated paper, comprising stretching an open-mesh fabric formed of unstrained rayon yarn having a substantial degree of extensibility to the extent that the individual yarns of the fabric are elongated to the point where their remaining extensibility is approximately equal to the extensibility of the paper with which the fabric is to be laminated, applying an aqueous adhesive to one face of each of two sheets of paper, introducing the fabric while in the above mentioned stretched condition between the adhesive coated faces of the sheets of paper whereby the fabric is wetted by the aqueous adhesive, and drying the adhesive and the fabric while maintaining the fabric in the stretched condition whereby the individual rayon yarns retain their elongation so long as they remain dry to thus produce a rayon fabric reinforced paper wherein the fabric and the paper have approximately the same extensibility.

2. The method of making a rayon fabric reinforced laminated paper, comprising stretching an open-mesh fabric formed of unstrained rayon yarn having a substantial degree of extensibility to the extent that the individual yarns of the fabric are elongated to the point where their remaining extensibility is approximately equal to the extensibility of the paper with which the fabric is to be laminated, applying an aqueous adhesive to one face of each of two sheets of paper, introducing the fabric while in the above mentioned stretched condition between the adhesive coated faces of the sheets of paper whereby the fabric is wetted by the aqueous adhesive, and applying heat and pressure to the outer faces of the sheets of paper to dry the adhesive and the fabric and maintain the fabric in the stretched condition during the drying whereby the individual rayon yarns of the fabric retain their elongation to thus produce a rayon fabric reinforced paper wherein the fabric and the paper have approximately the same extensibility.

#### References Cited in the file of this patent

#### UNITED STATES PATENTS

- |           |                    |               |
|-----------|--------------------|---------------|
| 2,503,024 | Boese et al. ----- | Apr. 4, 1950  |
| 2,575,666 | Knudson -----      | Nov. 20, 1951 |
| 2,674,555 | Pahl et al. -----  | Apr. 6, 1954  |

#### FOREIGN PATENTS

- |         |                     |               |
|---------|---------------------|---------------|
| 438,786 | Great Britain ----- | Nov. 21, 1935 |
| 148,830 | Australia -----     | Oct. 29, 1952 |